# EUROPEAN PATENT SPECIFICATION

(11) **EP 0 316 980 B1**
(45) Date of publication and mention of the grant of the patent: **23.06.1993**
(21) Application number: 88202408.6
(22) Date of filing: 28.10.1988
(51) Int. Cl.: G03C 1/72

(54) **Photochromatic composition and photochromatic articles which contain it**
Photochromische Zusammensetzung und diese Zusammensetzung enthaltende Gegenstände
Composition photochrome et articles à base de cette composition

(30) Priority: 05.11.1987 IT 2252887
(43) Date of publication of application: 24.05.1989
(73) Proprietor: ENICHEM SYNTHESIS S.p.A., 90139 Palermo (IT)
(72) Inventor: Casilli, Nicola, I-48100 Ravenna (IT); Crisci, Luciana, I-20079 Sant'Angelo Lodigiano, Milan (IT); Renzi, Fiorenzo, I-20064 Gorgonzola, Milan (IT); Rivetti, Franco, I-36015 Schio, Vicenza (IT)
(74) Representative: Fusina, Gerolamo

(56) References cited:
- EP-A- 0 195 898
- EP-A- 0 245 020
- US-A- 4 342 668

## Description

The present invention relates to a photochromatic composition which contains at least two organic photochromatic compounds.

The photochromatic compounds are substances which display the characteristics of reversibly changing in colour and/or degree of light transmission when they are exposed to some types of electromagnetic radiation, and to sun light, turning back into their original colour and transmission status when the initial light source is removed.

The substances endowed with photochromatic characteristics known from the prior art are many, and belong to several classes of both inorganic and organic compounds, as described, e.g., in "Photochromism", G.H. Brown (Ed.), Vol. IV, from the Weisseberger Series "Techniques of Organic Chemistry", Wiley-Interscience, New York (1971).

Among the organic photochromatic compounds, in particular those belonging to the class of the spiro-indolino-naphtho-oxazines are known, which are capable of conferring photochromatic characteristics on polymerized and transparent organic materials (organic glasses), for their use as sun filters and photochromatic optical articles, such as disclosed, e.g., in the following patents: US 3,562,172; US 3,578,602; US 4,215,010; US 4,342,668; EP 146 135, WO 85/02619; EP 245 020; and in European patent applications publ. Nos. 134,633 and 141,407.

The known photochromatic compounds belonging to the class of the spiro-indolino-naphtho-oxazines exhibit, as compared to other known organic photochromatic compounds (e.g., those belonging to the class of the spiro-piranes) the advantage of having a much higher fatigue strength, when they are submitted to repeated cycles of colouring and de-colouring; and a much higher ageing resistance when they are exposed to sun light, or to artificial ageing tests. This behaviour is very advantageous for the above set out uses.

However, the organic photochromatic compounds known from the prior art are practically colourless in their deactivated status, both in solution in common organic solvents, as well as when they are incorporated in transparent polymeric materials, and turn to a generally blue colour when they are activated. This blue colour is a disadvantage for their use as optical photochromatic articles, in particular in the ophthalmic sector, for which more neutral colours please, e.g., the gray colour.

Furthermore, the photochromatic effect obtained is in many cases of low intensity as regards the change in transmittance in the visible wavelength range. In other cases, such a change, although is satisfactory at low temperatures, is depressed down to unacceptedly low values with increasing temperature, even if within the values as required in practical use. Finally, the activation of the spiro-indolino-naphtho-oxazines, obtained under controlled laboratory conditions by irradiation with UV light of several wavelengths from about 320 to about 380 nm, is often not reproduced with the same satisfactory intensity when the exposure is carried out to the spectrum of frequencies and of relative intensities of sunlight, as required for the ophthalmic use, and as sun filter.

The purpose of the present invention is overcoming the drawbacks which affect the prior art by means of a novel photochromatic composition containing at least two photochromatic compounds belonging to the class of the spiro-indolino-naphtho-oxazines.

In accordance therewith, the present invention relates to a photochromatic composition consisting of at least two photochromatic compounds, both of which can be represented by the following general formula (I): wherein:
R₁ and R₂ independently represent a hydrogen atom or an atom of a halogen selected from F, CI
and Br, or a group selected from: (C₁-C₅)-alkoxy, nitro, cyano, and a linear or branched (C₁-C₅)-alkyl, either unsubstituted or substituted by a halogen atom selected from F, CI and Br, or (C₁-C₅)-alkoxy, (C₁-C₅)-alkylthio, (C₁-C₅)-carboxyalkyl, and cyano groups, or R₁ and R₂, when are not hydrogen, can be linked to any of the 4-, 5-, 6- and 7- positions of the indolinic moiety;
R₃ and R₄ independently represent linear or branched (C₁-C₅)-alkyl group, phenyl or benzyl ; or
R₃ and R₄, when considered jointly together with the carbon atom to which they are linked, form a (C₅-C₈)-cycloalkyl group;
R₅ is a phenyl, benzyl, allyl group, or a linear or branched (C₁-C₅)-alkyl group, either unsubstituted or substituted with at least one halogen atom selected from F, CI or Br, or (C₁-C₅)-alkoxy, (C₁-C₅)-alkylthio, (C₁-C₅)carboxyalkyl and cyano groups;
R₆ represents a hydrogen atom, a halogen selected from F, CI and Br, or a group selected from (C₁-C₅)-alkoxy, (C₁-C₅)-alkylthio, (C₁-C₅)-carboxyalkyl and cyano groups; and a linear or branched (C₁-C₅)-alkyl group, either unsubstituted or substituted with at least one halogen atom selected from F, CI and Br, or (C₁-C₅)-alkoxy, (C₁-C₅)-alkylthio, (Ci-C₅)-carboxyalkyl and cyano groups; or represents a condensed aromatic or heterocyclic ring;
R₆ when it does not represent hydrogen, or a condensed aromatic or heterocyclic ring, can be in any one of the 8'-, 9'-, 10' positions of the naphthenic moiety;
R₇ represents either a hydrogen atom or an and
R₈ and Rg represent, independently from each other, a hydrogen atom, or a linear or branched (C₁-C₅)-alkyl group, phenyl or benzyl; or
R₈ and Rg, when considered jointly together with the nitrogen atom to which they are linked, form a mono-cyclic or poly-cyclic structure, of from 5 to 12 members, possibly containing a further heteroatom selected from between oxygen and nitrogen; and
X represents either -CH- or N;
   in which composition at least one of the photochromatic compounds having formula (I) is characterized in that it has the R₇ substituent constituted by hydrogen, and at Least one of the photochromatic compounds having formula (I) is characterized in that it has the R₇ substituent constituted by a group wherein R₈ and Rg have the above seen meanings.

In the preferred form of practical embodiment, the photochromatic compounds of the composition according to the present invention, all of which can be defined by means of the general formula (I), and with the proviso that in at least one of them the R₇ substituent represents a hydrogen atom and in at least one of them the R₇ substituent represents the amino group the R₁, R₂, R₃, R₄, Rₛ, R₆ and, if present, R₈ and Rg, substituents, have the following meaning:
R₁ and R₂ independently represent the hydrogen atom, or the methyl, methoxy or halogen groups;
R₃ and R₄ represent each the methyl or ethyl group, or, when considered jointly, represent the cyclohexyl group;
R₅ represents a (C₁-C₅)-alkyl group;
R₆ represents the hydrogen atom or the methoxy group;
R₈ and R₉ jointly represent, together with the nitrogen atom to which they are linked, the piperidino, morpholino, pyrrolidinyl or hexamethyleneimino group; and
X represents either -CH- or N.
   Furthermore, still in the preferred form of practical embodiment, the Ri, R₂ and R₆ groups, when they do not represent hydrogen, or, in case of R₆ group, a ring structure, are respectively linked to the (4,5)- or (5,6)- and 9'-positions of the molecule.

Specific examples of photochromatic compounds in which the R₇ substituent is different from hydrogen, are:
A) 1,3,3-Trimethyl-6'-piperidino-spiro-[indolino-2,3'-(3H)-naphtho-(2,1-b)-(1,4)-oxazine].
B) 1,3,3-trimethyl-6'-morpholino-spiro[indolino-2,3'-(3H)-naphtho-(2,1-b)-(1,4)-oxazine].
C) 1,3,3,4,5,-(or 1,3,3,5,6)-pentamethy!-6'-p!per!d!no-sp!ro-[!ndo!!no-2,3'-(3H)-naphtho-(2,1 -b)-(1,4)-oxazine].
D) 1,3,3-trimethyl-6'-piperidino-9'-methoxy-spiro-[indolino-2,3'-(3H)-naphtho-(2,1-b)-(1,4)-oxazine]. Specific examples of photochromatic compounds in which the R₇ substituent is hydrogen are:
E) 1,3,3,4,5- (or 1,3,3,5,6) pentamethyl-spiro-[indolino-2,3'-(3H)-naphtho-(2,1-b)-(1,4)-oxazine].
F) 1,3,3-trimethyl-spiro-[indolino-2,3'-(3H)-naphtho-(2,1-b)-(1,4)-oxazine].
G) 1,3,3-trimethyl-9'-methoxy-spiro-[indolino-2,3'-(3H)-naphtho-(2,1-b)-(1,4)-oxazine].

The above listed photochromatic compounds have been incorporated into transparent organic polymers by means of techniques depending on the polymer used.

In the photochromatic mixture of the present invention, the simultaneous presence of a photochromatic compound definable by means of formula (I) and having an -NR8R9 in the 6'-position of the molecule, and of a photochromatic compound definable by means of said formula, but in which the substituent in 6'- position is hydrogen atom, is advantageous.

In such a mixture, as said, both compounds act with a synergistic effect on the regulation of the sun light, generating a more intense colour, and with shorter response times, than the normal photochromatic organic compounds of the prior art, as well as than the individual components of the same mixture.

The change in transmittance is furthermore maintained at satisfactory values with increasing room temperature, and much higher than as required by the practical application. Furthermore, the shades of colour which can be obtained by means of the use of the photochromatic mixture of the present invention are more neutral than the blue colour generally shown by individual components, and can be modulated within a wide range by means of a properly balanced dosage of both basic components, as well as of other components known from the prior art.

Advantageously, this mutual mol ratio of the two photochromatic components defined by the general formula (I) and respectively bearing the -NR8R9 group and hydrogen in the 6'-position, is a number comprised within the range of from 0.1 and 9 and preferably from 0.2 to 1.5.

As said, the photochromatic mixture of the present invention can be constituted by more than two compounds as defined by the general formula (I), provided that at least two of them are different from each other as to the 6'-substituent, as above said.

Said mixtures can furthermore additionally contain other components, such as the U.V. stabilizers known from the prior art, capable of improving the duration of the photochromatic effect, without impairing the intensity of photocolourability of the same mixtures. Non-limitative examples of U.V.-stabilizers for the purposes of the present invention are the hindered ammines (HALS).

The photochromatic mixture according to the present invention is useful in the production of photochromatic articles endowed with particular colour transitions, a high activation by exposure to sun light, a high fatigue and ageing resistance.

The photochromatic mixture according to the present invention is applied to the surface of, or is incorporated into, the desired articles, generally constituted by transparent polymeric materials, by means of suitable techniques. Photochromatic polymeric articles can be obtained by means of moulding techniques (e.g., injection-moulding, press-moulding, and so forth;) by homogeneously dispersing throughout the mass of the photochromatic mixture.

According to an alternative route, the mixture can be dissolved in a suitable solvent, together with a polymeric material (e.g., poly-methyl-methacrylate, polyvinyl-alcohol, polyvinyl pyrrolidone, poly-vinylbutyral, cellulose acetate-butyrate or epoxy resin, polysiloxane resin or urethan resin, and so forth), and deposited on a transparent support in order to form, after the evaporation of the solvent, a photochromatic coating.

According to an alternative route, the photochromatic mixture can be added to a polymerizable monomer, e.g., methyl-methacrylate, so that after a polymerization carried out in the presence of a suitable polymerization initiator, e.g., azo-bis(isobutyronitrile), it results to be evenly incorporated to the formed resin.

According to an alternative route, the photochromatic mixture can be dissolved in a suitable solvent, in the presence of a resin, as above disclosed, and from this solution, by evaporating the solvent, a photochromatic film or sheet can be formed, which contain the uniformly dispersed photochromatic mixture.

According to an alternative route, the photochromatic mixture can be applied to a transparent substrate (e.g., a polycarbonate substrate, a polymethyl-methacrylate substrate or a poly-diethylene-glycol-bis(allyl carbonate) substrate) by means of a surface impregnation obtained by placing the substrate into contact, at a suitable temperature, with a solution or dispersion which contains the mixture.

In particular, by means of the above disclosed techniques, photochromatic articles can be obtained, such as photochromatic ophthalmic lenses and photochromatic sun filters, that is to say, which are capable of constituting an at least partial screen towards the sun radiation, in a reversible way.

Such articles can be advantageously used, e.g., as lenses for sun glasses, prescription-lenses, contact lenses, glasses for cars or transport means in general, and windows in the building sector.

The following experimental examples are reported in order to illustrate the present invention without limiting it. The compounds reported in the Examples were prepared according to methods known from the prior art.

In particular, optical photochromatic articles of polymethyl-methacrylate (PMMA) were obtained by adding the photochromatic compound and the polymerization initiator azo-bis(isobutyro-nitrile) (AIBN) to the monomer and then carrying out the polymerization by casting into moulds of a suitable shape.

Optical articles of poly-diethylene-glycol-bis(allyl-carbonate) were made photochromatic by means of a surface impregnation technique. For that purpose, a solution or suspension is prepared of the photochromatic compound in a suitable solvent or dispersant, normally selected from among the usual organic solvents, silicone oils, fluorinated oils, and the like, and the photochromatic compound is transferred on to the polymeric substrate by dipping the polymeric article in said solution or suspension, for suitable times and at suitable temperatures.

A more detailed disclosure of the application processes used is given in the hereinunder reported experimental examples.

On the optical photochromatic articles obtained, the following characteristics are determined:
- The U.V.-visible spectrum in the deactivated status (optical density at Xₘₐₓ), as determined by the Cary 2300 spectrophotometer.
- The change in light transmittance ( A Y) at 23 _{°} C, as determined by the MACBETH spectrophotometer, after a 120-second activation with an UV-A lamp of 9 W/m² of irradiance. The values of A Y were also measured after a 4-minute exposure to sun light, by using the Gardner's Hazemeter XL 211.
- Kinetics of return to the deactivated form (time for recovery of 50% of the initial transmittance, t_{1/2}), by means of a MACBETH spectrophotometer, under the same activation conditions as hereinabove disclosed.
- Ageing resistance, as determined by means of an Atlas Weather-O-Meter equipped with a continous- irradiation xenon lamp of 6,500 W, operating at a temperature of 63 _{°} C on the reference black panel, and at a relative humidity of 50%. The ageing resistance is evaluated by measuring, after various times of exposure in the Weather-O-Meter, the values of optical density at Xₘₐₓ of the deactivated form, and the residual value of A Y after activation with the UV-A lamp.

### Example 1

Photochromatic lenses of poly-diethylene-glycol-bis(allyl-carbonate) are prepared by means of surface impregnation with mixtures of (A) and (E) photochromatic compounds in the following proportions:

In particular, a dispersion of 2% by weight of said (a), (b) or (c) mixture in silicone oil is prepared.

In order to transfer the photochromatic compound, the lens is dipped into the siliconic dispersion for times ranging from 30 to 90 minutes, and at temperatures comprised within the range of from 170 to 190°C, as a function of the desired value for optical density. At the end of the impregnation, the lens is washed with petroleum ester, and the characteristics as listed hereinabove in the specification are evaluated.

The results relevant to the (a), (b) and (c) photochromatic mixtures are reported in Table (I), as compared to those obtained on a lens obtained, under the same conditions, by using the (A) photochromatic compound alone.

In Table II, the results obtained from the accelerated ageing tests in W-O-M are reported

From an examination of these results, it is clear that the (a), (b) and (c) mixtures, with the photochromatic activity (Δ Y), and the return times back to the deactivated status (t½), being the same, show, as compared to the individual photochromatic (A) and (E) products, the advantages of a colour of the activated status which is more neutral, and can be modulated as a function of their ratio by weight; a considerably higher ageing strength and photochromatic activity then the pure (A) product, and the pure (E) product, respectively.

### Example 2

The photochromatic response to sun light exposure is evaluated of a neutral lens of poly-diethyleneglycol-bis(allyl carbonate) impregnated with the (b) photochromatic mixture of Example 1, as compared to a similar lens impregnated with the spiro-oxazinic photochromatic compound known from the prior art, having the formula: wherein the two methyl groups on the benzene-indolinic ring are in the 4,5- and 5,6-positions.

Both of them were activated by a 4-minute exposure to sun light, and were evaluated for the change in light transmittance (A Y) shown by the two lenses following said exposure, and measured by means of the Gardner's Hazegard XL 211.

The results are reported in Table III.

As compared to the lens with the spiro-oxazine known from the prior art, the lens obtained with the (b) photochromatic mixture of the present invention shows a more neutral colour of the activated status, a higher photochromatic activity (A Y), and a twice as high return rate to the deactivated status

### Example 3

With the (b) photochromatic mixture of the previous example, a neutral photochromatic lens of poly-(methyl-methacrylate) is prepared, which has the following composition:
- (b) photochromatic mixture 10 mg 0.066 parts
- MethyL-methacryLate 15 g 100 parts
- Azo-bis(isobutyro-nitrile) 0.15 g 0.100 parts

The polymerization of the lens is carried out by casting, maintaining the mould in a temperature- controlled water bath at 55 °C for 80 hours.

At the end of the polymerizazion, by opening the mould, a photochromatic lens of poly(methyl methacrylate) is obtained, which has the characteristics as reported in Tables IV and V.

In the same tables, also the characteristics are reported for comparison purposes, of lenses obtained, with the other conditions being the same, by separately using the individual (A) and (E) photochromatic compounds.

These results demonstrate that in poly-(methyl-methacrylate), the (b) composition according to the present invention unexpectedly shows photochromatic characteristics as well a stability, which are similar to those of the pure (A) photochromatic compound, even if it is constituted for its major portion by the (E) photochromatic compound, which, in the pure state, displays very bad photochromatic characteristics and ageing resistance.

### Example 4

A mixture is prepared, which is constituted by a polypropylene powder of MOPLEN FLF 20 type, having a fluidity degree of 11, manufactured by HIMONT, and by the (b) photochromatic mixture of Example 1, in the mutual ratio by weight to each other of respectively 100:0.25.

For comparison purposes, mixtures of polypropylene with the individual (A) and (E) photochromatic compounds in the same weight ratios are prepared.

Said polymeric mixtures are transformed into films of 50 m of thickness by extrusion at the temperature of 215°C. The photochromatic characteristics of the so-obtained films, and the relevant resistances under such conditions as reported in the text, are reported in Table VI.

### Example 5

A mixture of the (D) and (G) photochromatic compounds in the weight ratio of 60/40 is prepared.

Said mixture is applied by surface impregnation to neutral lenses of poly-diethylene-glycol-bis(allyl carbonate), and is evaluated as disclosed at Example 1.

The results are reported in Table VII.

### Example 6

The following mixtures with a different weight ratio between the photochromatic compounds (A) and (F) are prepared:

The mixtures Nos. 1 and 5, are reported for comparative purposes.

Said mixtures were applied to the surface of neutral lenses of poly-diethylene-glycol-bis(allyl carbonate) according to the same technique as reported in Example 1.

The resulting properties are reported in Table VIII.

The reported data shows the synergistic effect of the two (A) and (F) products, in that the photochromatic activity of their mixtures is very close to the photochromatic activity displayed by the more active (A) compound alone, and the times of return back to the deactivated form are considerably shorter.

The structures of a few photochromatic compositions of the invention are graphically illustrated in the accompagying drawings, wherein:
Figure 1 is an NMR¹H spectrogram of the photochromatic compound (A) at 10-5 δ;
Figure 2 is a spectrogram similar to that of Figure 1, but taken at 5-0 δ;
Figure 3 is an NMR¹H spectrogram of the photochromatic composition (B);
Figure 4 is an NMR¹H spectrogram of the photochromatic composition (C), and
Figure 5 is an NMR¹H spectrogram of the photochromatic composition (D).

For all the NMR¹H spectrograms shown in Figures 1-5, the substances to be tested were dissolved in deuterated chloroform.

## Claims (Claims for the following Contracting State(s) : AT, BE, CH, DE, FR, GB, GR, IT, LI, LU, NL, SE)

1. Photochromatic composition of at least two photochromatic compounds, both of which can be represented by the following general formula (I): wherein:
R₁ and R₂ independently represent a hydrogen atom or an atom of a halogen selected from F, CI and Br, or a group selected from: (C₁-Cₛ)-alkoxy, nitro, cyano, and a linear or branched (C₁-C₅)-alkyl, either unsubstituted or substituted by a halogen atom selected from F, CI and Br, or (C₁-C₅ )-alkoxy, (C₁-C₅)-alkylthio, (C₁-Cₛ)-carboxyalkyl, and cyano groups;
R₃ and R₄ independently represent linear or branched (C₁-C₅)-alkyl group, phenyl or benzyl; or
R₃ and R₄, when considered jointly together with the carbon atom to which they are linked, form a (C₅-C₈)-cycloalkyl group;
R₅ is a phenyl, benzyl, allyl group, or a linear or branched (C₁-C₅)-alkyl group, either unsubstituted or substituted with at least one halogen atom selected from F, CI or Br, or (C₁-C₅)-alkoxy, (C₁-C₅)-alkylthio, (C₁-C₅)carboxyalkyl and cyano groups;
R₆ represents a hydrogen atom, a halogen selected from F, CI and Br, or a group selected from (C₁-C₅)-alkoxy, (C₁-C₅ )-alkylthio, (C₁-C₅ )-carboxyalkyl and cyano groups; and a linear or branched (C₁-C₅)-alkyl group, either unsubstituted or substituted with at least one halogen atom selected from F, CI and Br, or (C₁-C₅)-alkoxy, (C₁-C₅)-alkylthio, (C₁-C₅)-carboxyalkyl and cyano groups; or represents a condensed aromatic or heterocyclic ring;
R₆ when it does not represent hydrogen, or a condensed aromatic or heterocyclic ring, can be in any one of the 8'-, 9'-, 10' positions of the naphthenic moiety;
R₇ represents either a hydrogen atom or an and
R₈ and Rg represent, independently from each other, a a hydrogen atom, or a linear or branched (C₁-C₅)-alkyl, phenyl, or benzyl group, or
R₈ and Rg, when considered jointly with the nitrogen atom to which they are linked, from a mono-cyclic or poly-cyclic structure, of from 5 to 12 members, possibly containing a further heteroatom selected from oxygen and nitrogen; and
X represents either a CH group or N; in which composition at least one of the photochromatic compounds defined by the formula (I) has the R7 substituent constituted by hydrogen, and at least one of the photochromatic compounds defined by the formula (I) has the R7 substituent constituted by a group wherein R₈ and Rg have the above stated meanings.

2. Photochromatic composition according to claim 1, characterized in that in at least one of the compounds defined in formula (I), the substituents:
R₁ and R₂ independently represent the hydrogen atom, or the methyl, or methoxy groups;
R₃ and R₄ represent each the methyl or ethyl group, or, when considered jointly, represent the cyclohexyl group;
R₅ represents a (C₁-C₅)-alkyl group;
R₆ represents the hydrogen atom or the methoxy group;
R₇ represents an -NR₈ R₉ group, wherein
R₈ and Rg jointly represent, together with the nitrogen atom they are linked to, the piperidino, morpholino, pyrrolidinyl or hexamethylene-imino groups; and
X represents either -CH- or N.

3. Photochromatic composition according to claims 1 and 2, characterized in that the ratio by moles of the photochromatic compounds defined by formula (I) wherein R₇ is an -NR₈R₉ group to the compounds, also defined by formula (I), wherein R₇ is hydrogen, is a number comprised within the range of from 0.1 to 9.

4. Photochromatic composition according to claims 1 and 2, characterized in that the ratio by moles of the photochromatic compounds defined by formula (I) wherein R₇ is an -NR₈R9 group to the compounds, also defined by formula (I), wherein R₇ is hydrogen, is a number comprised within the range of from 0.2 to 1.5.

5. Photochromatic composition according to Claim 1, or 2, or 3, or 4, containing 1,3,3-trimethyl-6'-piperidino-spiro-[indolino-2,3'-(3H)-naphtho-(2,1-b)-(1,4)-oxazine].

6. Photochromatic composition according to claims from 1 to 4, containing 1,3,3-trimethyl-6'-morpholino- spiro-[indolino-2,3'-(3H)-naphtho-(2,1 -b)-(1,4)-oxazine].

7. Photochromatic composition according to claims from 1 to 4, containing 1,3,3,4,5,- (or 1,3,3,5,6-) pentamethyl-6'-piperidino-spiro-[indolino-2,3'-(3H)-naphtho-(2,1-b)-(1,4)-oxazine].

8. Photochromatic composition according to claims from 1 to 4, containing 1,3,3-trimethyl-6'-piperidino-9'-methoxy-spiro-[indolino-2,3'-(3H)-naphtho-(2,1-b)-(1,4)-oxazine].

9. Photochromatic composition according to claims from 1 to 4, containing 1,3,3,4,5- (or 1,3,3,5,6-) pentamethyl-spiro-[indolino-2,3'-(3H)-naphtho-(2,1-b)-(1,4)-oxazine].

10. Photochromatic composition according to claims from 1 to 4, containing 1,3,3-trimethyl-spiro-[indolino-2,3'-(3H)-naphtho-(2,1 -b)-(1,4)-oxazine].

11. Photochromatic composition according to claims from 1 to 4, containing 1,3,3-trimethyl-9'-methoxy- spiro-[indolino-2,3'-(3H)-naphtho-(2,1 -b)-(1,4)-oxazine].

12. Photochromatic composition according to the preceding claims, further comprising an U.V.- stabilizer.

13. Photochromatic composition according to claims 12, characterized in that the U.V.-stabilizer is a sterically hindered amine (HALS).

14. Photochromatic article comprising a transparent organic polymer, and containing on its surface, or inside its mass, a photochromatic composition according to claims from 1 to 10.

15. Photochromatic article according to claim 14, wherein said transparent organic polymer is selected from poly-methyl-methacrylate, polyvinyl-alcohol, polyvinyl butyral, polyvinyl-pyrrolidone, cellulose acetate-butyrate, epoxy resins, polysiloxane resins, polyurethan resins, polycarbonate and poly- diethylene-glycol bis(allyl carbonate).

## Claims (Claims for the following Contracting State(s) : ES)

1. Process for preparing a photochromatic composition characterized by comprising the step of combining at least two photochromatic compounds, both of which can be represented by the following general formula (I): wherein:
R₁ and R₂ independently represent a hydrogen atom or an atom of a halogen selected from F, CI and Br, or a group selected from: (C₁-Cₛ)-alkoxy, nitro, cyano, and a linear or branched (C₁-C₅)-alkyl, either unsubstituted or substituted by a halogen atom selected from F, CI and Br, or (C₁-C₅ )-alkoxy, (C₁-C₅ )-alkylthio, (C₁-Cₛ)-carboxyalkyl, and cyano groups;
R₃ and R₄ independently represent linear or branched (C₁-C₅)-alkyl group, phenyl or benzyl; or
R₃ and R₄, when considered jointly together with the carbon atom to which they are linked, form a (C₅-C₈)-cycloalkyl group;
R₅ is a phenyl, benzyl, allyl group, or a linear or branched (C₁-C₅)-alkyl group, either unsubstituted or substituted with at least one halogen atom selected from F, CI or Br, or (C₁-C₅)-alkoxy, (C₁-C₅)-alkylthio, (C₁-C₅)carboxyalkyl and cyano groups;
R₆ represents a hydrogen atom, a halogen selected from F, CI and Br, or a group selected from (C₁-C₅)-alkoxy, (C₁-C₅)-alkylthio, (C₁-C₅)-carboxyalkyl and cyano groups; and a linear or branched (C₁-C₅)-alkyl group, either unsubstituted or substituted with at least one halogen atom selected from F, CI and Br, or (C₁-C₅)-alkoxy, (C₁-C₅)-alkylthio, (C₁-C₅)-carboxyalkyl and cyano groups; or represents a condensed aromatic or heterocyclic ring;
R₆ when it does not represent hydrogen, or a condensed aromatic or heterocyclic ring, can be in any one of the 8'-, 9'-, 10' positions of the naphthenic moiety;
R₇ represents either a hydrogen atom or an and
R₈ and Rg represent, independently from each other, a a hydrogen atom, or a linear or branched (C₁-C₅)-alkyl, phenyl, or benzyl group, or
R₈ and Rg, when considered jointly with the nitrogen atom to which they are linked, from a mono-cyclic or poly-cyclic structure, of from 5 to 12 members, possibly containing a further heteroatom selected from oxygen and nitrogen; and
X represent either a CH group or N;
in which composition at least one of the photochromatic compounds defined by the formula (I) has the R₇ substituent constituted by hydrogen, and at least one of the photochromatic compounds defined by the formula (I) has the R₇ substituent constituted by a group wherein R8 and R9 have the above stated meanings.

2. Process according to claim 1, characterized in that in at least one of the compounds defined in formula (I), the substituents:
R₁ and R₂ independently represent the hydrogen atom, or the methyl, or methoxy groups;
R₃ and R₄ represent each the methyl or ethyl group, or, when considered jointly, represent the cyclohexyl group;
R₅ represents a (C₁-C₅)-alkyl group;
R₆ represents the hydrogen atom or the methoxy group;
R₇ represents an -NR₈R₉ group, wherein
R₈ and Rg jointly represent, together with the nitrogen atom they are linked to, the piperidino, morpholino, pyrrolidinyl or hexamethyleneimino groups; and
X represents either CH or N.

3. Process according to claims 1 and 2, characterized in that the ratio by moles of the photochromatic compounds defined by formula (I) wherein R₇ is an -NR₈R₉ group to the compounds, also defined by formula (I), wherein R₇ is hydrogen, is a number comprised within the range of from 0.1 to 9.

4. Process according to claims 1 and 2, characterized in that the ratio by moles of the photochromatic compounds defined by formula (I) wherein R₇ is an -NR₈Rg group to the compounds, also defined by formula (I), wherein R₇ is hydrogen, is a number comprised within the range of from 0.2 to 1.5.

5. Process according to Claim 1, or 2, or 3, or 4, characterized in that the composition contains: 1,3,3-trimethy!-6'-piperidino-spiro-[indo!ino-2,3'-(3H)-naphtho-(2,1 -b)-(1,4)-oxazine].

6. Process according to Claims 1 to 4, characterized in that the composition contains:
1,3,3-trimethyl-6'-morpholino-spiro-[indolino-2,3'-(3H)-naphtho-(2,1 -b)-(1,4)-oxazine].

7. Process according to Claims 1 to 4, characterized in that the composition contains:
1,3,3,4,5-(or 1,3,3,5,6-)-pentamethyl-6'-piperidino-spiro [indolino-2,3'-(3H)-naphtho-(2,1-b)-(1,4)-oxazine].

8. Process according to to Claims 1 to 4, characterized in that the composition contains: 1,3,3-trimethyl-6'-piperidino-9'-methoxy-spiro-[indolino-2,3'-(3H)-naphtho-(2,1-b)-(1,4)-oxazine].

9. Process according to Claims 1 to 4, characterized in that the composition contains:
1,3,3,4,5- (or 1,3,3,5,6-) pentamethyl-spiro-[indolino-2,3'-(3H)-naphtho-(2,1-b)-(1,4)-oxazine].

10. Process according to Claims 1 to 4, characterized in that the composition contains: 1,3,3-trimethy!-spiro-[indo!ino-2,3'-(3H)-naphtho-(2,1 -b)-(1,4)-oxazine].

11. Process according to Claims 1 to 4, characterized in that the composition contains: 1,3,3-trimethyl-9'-methoxy-spiro-[indolino-2,3'-(3H)-naphtho-(2,1 -b)-(1,4)-oxazine].

12. Process according to Claim 1, characterized in that it further comprises the addition of a UV-stabilizer.

## Patentansprüche (Patentansprüche für folgende(n) Vertragsstaat(en) : AT, BE, CH, DE, FR, GB, GR, IT, LI, LU, NL, SE)

1. Photochrome Zusammensetzung aus wenigstens zwei photochromen Verbindungen, wovon beide durch die folgende allgemeine Formel (I) wiedergegeben werden können: worin:
R₁ und R₂ unabhängig voneinander für ein Wasserstoffatom oder ein Halogenatom, ausgewählt aus F, CI und Br, oder eine Gruppe, ausgewählt aus (C₁-C₅)-Alkoxy, Nitro, Cyano und einem linearen oder verzweigten (C₁-C₅)-Alkyl, entweder unsubstituiert oder substituiert mit einem Halogenatom, ausgewählt aus F, CI und Br, oder (C₁-C₅)⁻Alkoxy, (C1-Cs)-Alkylthio, (C₁-C₅)-Carboxyalkyl, und Cyanogruppen bestehen;
R₃ und R₄ unabhängig voneinander für eine lineare oder verzweigte (C₁-C₅)-Alkylgruppe, Phenyl oder Benzyl stehen; oder
R₃ und R₄ bilden eine (C₅-C₈)-Cycloalkylgruppe, wenn sie zusammen mit dem Kohlenstoffatom, an das sie gebunden sind, betrachtet werden;
R₅ ist eine Phenyl-, Benzyl-, Allylgruppe oder eine lineare oder verzweigte (C₁-C₅)-Alkylgruppe, entweder unsubstituiert oder substituiert mit wenigstens einem Halogenatom, ausgewählt aus F, CI oder Br, oder (C₁-C₅)-Alkoxy-, (C₁-C₅)-Alkylthio-, (C₁-C₅)-Carboxyalkyl- und Cyanogruppen;
R₆ für ein Wasserstoffatom steht, ein Halogen, ausgewählt aus F, CI und Br, oder eine Gruppe, ausgewählt aus (C₁-C₅)-Alkoxy-, (C₁-C₅)-Alkylthio-, (C₁-C₅)-Carboxyalkyl- und Cyanogruppen, und eine lineare oder verzweigte (C₁-C₅)-Alkylgruppe, entweder unsubstituiert oder substituiert mit wenigstens einem Halogenatom, ausgewählt aus F, CI und Br, oder (C₁-Cs)-Alkoxy-, (C₁-C₅)-Alkylthio-, (C₁-C₅)-Carboxyalkyl- und Cyanogruppen; oder für einen kondensierten aromatischen oder heterocyclischen
Ring steht;
R₆ kann, wenn es nicht für Wasserstoff oder einen kondensierten aromatischen oder heterocyclischen
Ring steht, an irgendeiner der 8'-, 9'-, 10'-Positionen des naphthenischen Teiles stehen;
R⁷ entweder für ein Wasserstoffatom oder steht; und
R₈ und Rg unabhängig voneinander für ein Wasserstofftom oder eine lineare oder verzweigte (C₁-C₅)-Alkyl-, Phenyl- oder Benzylgruppe stehen, oder
R₈ und Rg bilden, wenn sie zusammen mit dem Stickstoffatom betrachtet werden, an das sie gebunden sind, eine monocyclische oder polycyclische Struktur mit 5 bis 12 Gliedern, möglicherweise enthaltend ein weiteres Heteroatom, ausgewählt aus Sauerstoff und Stickstoff; und
X entweder für eine CH-Gruppe oder N steht, wobei in dieser Zusammensetzung wenigstens eine der photochromen Verbindungen, definiert durch die Formel (I), einen R₇-Substituentenhat, der aus Wasserstoff besteht, und wenigstens eine der photochromen Verbindungen, definiert durch die Formel (I), einen R₇-Substituenten hat, bestehend aus der Gruppe worin R₈ und Rg die oben angegebenen Bedeutungen haben.

2. Photochrome Zusammensetzung nach Anspruch 1, dadurch gekennzeichnet, daß in wenigstens eine der Verbindungen, definiert nach Formel (I), die Substituenten
R₁ und R₂ unabhängig voneinander für das Wasserstoffatom oder Methyl oder Methoxygruppe stehen;
R₃ und R₄ jeweils für die Methyl- oder Ethylgruppe oder, wenn sie zusammen betrachtet werden, für die Cyclohexylgruppe stehen;
R₅ für eine (C₁-C₅)-Alkylgruppe steht;
R₆ für das Wasserstoffatom oder die Methoxygruppe steht;
R₇ für eine -NR₈ R₉-Gruppe steht, worin
R₈ und Rg zusammen, verknüpft mit dem Stickstoffatom, an das sie gebunden sind, für die Piperidino-, Morpholino, Pyrrolidinyl- oder Hexamethyleniminogruppen stehen; und
X entweder für CH oder N steht.

3. Photochrome Zusammensetzung nach den Ansprüchen 1 und 2, dadurch gekennzeichnet, daß das Molverhältnis der nach Formel (I) definierten photochromen Verbindungen, worin R₇ eine -NR₈R₉-Gruppe zu den Verbindungen ist, ebenfalls definiert durch die Formel (I), worin R₇ Wasserstoff ist, durch eine Zahl innerhalb des Bereichs von 0,1 bis 9 umfaßt wird.

4. Photochrome Zusammensetzung nach Anspruch 1 und 2, dadurch gekennzeichnet, daß das Molverhältnis der photochromen Verbindungen, definiert durch Formel (I), worin R₇ eine -NR₈R₉-Gruppe ist, zu den Verbindungen, ebenfalls definiert durch die Formel (I), worin R₇ Wasserstoff ist, durch eine Zahl innerhalb des Bereichs von 0,2 bis 1,5 umfaßt wird.

5. Photochrome Zusammensetzung nach Anspruch 1 oder 2 oder 3 oder 4, enthaltend 1,3,3-Trimethyl-6'-piperidino-spiro-[indolino-2,3'-(3H)-naphtho-(2,1-b)-(1,4)-oxazin].

6. Photochrome Zusammensetzung nach den Ansprüchen 1 bis 4, enthaltend 1,3,3-Trimethyl-6'-morpholino-spiro-[indolino-2,3'-(3H)-naphtho-(2,1-b)-(1,4)-oxazin].

7. Photochrome Zusammensetzung nach den Ansprüchen 1 bis 4, enthaltend 1,3,3,4,5-(oder 1,3,3,5,6- )Pentamethyl-6'-piperidino-spiro-[indolino-2,3'-(3H)-naphtho-(2,1-b)-(1,4)-oxazin].

8. Photochrome Zusammensetzung nach den Ansprüchen 1 bis 4, enthaltend 1,3,3-Trimethyl-6'-piperidino-9'-methoxy-spiro-[indolino-2,3'-(3H)-naphtho-(2,1-b)-(1,4)-oxazin].

9. Photochrome Zusammensetzung nach den Ansprüchen 1 bis 4, enthaltend 1,3,3,4,5-(oder 1,3,3,5,6- )Pentamethyl-spiro-[indolino-2,3'-(3H)-naphtho-(2,1-b)-(1,4)-oxazin].

10. Photochrome Zusammensetzung nach den Ansprüchen 1 bis 4, enthaltend 1,3,3-Trimethyl-spiro-[indolino-2,3'-(3H)-naphtho-(2,1 -b)-(1,4)-oxazin].

11. Photochrome Zusammensetzung nach den Ansprüchen 1 bis 4 enthaltend 1,3,3-Trimethyl-9'-methoxy- spiro-[indolino-2,3'-(3H)-naphtho-(2,1 -b)-(1,4)-oxazin].

12. Photochrome Zusammensetzung nach den vorhergehenden Ansprüchen, weiterhin umfassend einen UV-Stabilisator.

13. Photochrome Zusammensetzung nach Anspruch 12, dadurch gekennzeichnet, daß der UV-Stabilisator ein sterisch gehindertes Amin (HALS) ist.

14. Photochromer Artikel, umfassend ein transparentes organisches Polymer und enthaltend auf seiner Oberfläche oder in der Masse eine photochrome Zusammensetzung nach den Ansprüchen 1 bis 10.

15. Photochromer Artikel nach Anspruch 14, worin das transparente organische Polymer ausgewählt ist aus Polymethylmethacrylat, Polyvinylalkohol, Polyvinylbutyral, Polyvinylpyrrolidon, Celluloseacetat-butyrat, Epoxyharzen, Polysiloxanharzen, Polyurethanharzen, Polycarbonat und Polydiethylenglykol-bis-(allylcarbonat).

## Patentansprüche (Patentansprüche für folgende(n) Vertragsstaat(en) : ES)

1. Verfahren zur Herstellung einer photochromen Zusammensetzung gekennzeichnet dadurch, daß der Schritt der Vereinigung von wenigstens zwei photochromen Verbindungen umfaßt wird, wobei beide davon durch die folgende allgemeine Formel (I) wiedergegeben werden können: worin:
R₁ und R₂ unabhängig voneinander für ein Wasserstoffatom oder ein Halogenatom, ausgewählt aus F, CI und Br, oder eine Gruppe, ausgewählt aus (C₁-C₅)-Alkoxy, Nitro, Cyano und einem linearen oder verzweigten (C₁-C₅)-Alkyl, entweder unsubstituiert oder substituiert mit einem Halogenatom, ausgewählt aus F, CI und Br, oder (C₁-Cₛ)-Alkoxy, (C1-Cs)-Alkylthio, (C₁-C₅)-Carboxyalkyl, und Cyanogruppen bestehen;
R₃ und R₄ unabhängig voneinander für eine lineare oder verzweigte (C₁-C₅)-Alkylgruppe, Phenyl oder Benzyl stehen; oder
R₃ und R₄ bilden eine (C₅-C₈)-Cycloalkylgruppe, wenn sie zusammen mit dem Kohlenstoffatom, an das sie gebunden sind, betrachtet werden;
R₅ ist eine Phenyl-, Benzyl-, Allylgruppe oder eine lineare oder verzweigte (C₁-C₅)-Alkylgruppe, entweder unsubstituiert oder substituiert mit wenigstens einem Halogenatom, ausgewählt aus F, CI oder Br, oder (C₁-C₅)-Alkoxy-, (C₁-C₅)-Alkylthio-, (C₁-C₅)-Carboxyalkyl- und Cyanogruppen;
R₆ für ein Wasserstoffatom steht, ein Halogen, ausgewählt aus F, CI und Br, oder eine Gruppe, ausgewählt aus (C₁-C₅)-Alkoxy-, (C₁-C₅)-Alkylthio-, (C₁-C₅)-Carboxyalkyl- und Cyanogruppen, und eine lineare oder verzweigte (C₁-C₅)-Alkylgruppe, entweder unsubstituiert oder substituiert mit wenigstens einem Halogenatom, ausgewählt aus F, CI und Br, oder (C₁-C₅)-Alkoxy, (C₁-C₅)-Alkylthio-, (C₁-C₅)-Carboxyalkyl- und Cyanogruppen; oder für einen kondensierten aromatischen oder heterocyclischen Ring steht;
R₆ kann, wenn es nicht für Wasserstoff oder einen kondensierten aromatischen oder heterocyclischen Ring steht, an irgendeiner der 8'-, 9'-, 10'-Positionen des naphthenischen Teiles stehen; R⁷ entweder für ein Wasserstoffatom oder steht; und
R₈ und Rg unabhängig voneinander für ein Wasserstofftom oder eine lineare oder verzweigte (C₁-C₅)-Alkyl-, Phenyl- oder Benzylgruppe steht, oder
R₈ und Rg bilden, wenn sie zusammen mit dem Stickstoffatom betrachtet werden, an das sie gebunden sind, eine monocyclische oder polycyclische Struktur mit 5 bis 12 Gliedern, möglicherweise enthaltend ein weiteres Heteroatom, ausgewählt aus Sauerstoff und Stickstoff; und
X entweder für eine CH-Gruppe oder N steht;
wobei in dieser Zusammensetzung wenigstens eine der photochromen Verbindungen, definiert durch die Formel (I), einen R₇-Substituentenhat, der aus Wasserstoff besteht, und wenigstens eine der photochromen Verbindungen, definiert durch die Formel (I), einen R₇-Substituenten hat, bestehend aus der Gruppe worin R₈ und Rg die oben angegebenen Bedeutungen haben.

2. Verfahren nach Anspruch 1, dadurch gekennzeichnet, daß in wenigstens eine der Verbindungen, definiert nach Formel (I), die Substituenten
R₁ und R₂ unabhängig voneinander für das Wasserstoffatom oder Methyl oder Methoxygruppe stehen;
R₃ und R₄ jeweils für die Methyl- oder Ethylgruppe oder, wenn sie zusammen betrachtet werden, für die Cyclohexylgruppe stehen;
R₅ für eine (C₁-C₅)-Alkylgruppe steht;
R₆ für das Wasserstoffatom oder die Methoxygruppe steht;
R₇ für eine -NR₈R₉-Gruppe steht, worin
R₈ und Rg zusammen, verknüpft mit dem Stickstoffatom, an das sie gebunden sind, für die Piperidino-, Morpholino, Pyrrolidinyl- oder Hexamethyleniminogruppen stehen; und
X entweder für CH oder N steht.

3. Verfahren nach Anspruch 1 und 2, dadurch gekennzeichnet, daß das Molverhältnis der nach Formel (I) definierten photochromen Verbindungen, worin R₇ eine -NR₈R₉-Gruppe zu den Verbindungen ist, ebenfalls definiert durch die Formel (I), worin R₇ Wasserstoff ist, durch eine Zahl innerhalb des Bereichs von 0,1 bis 9 umfaßt wird.

4. Verfahren nach Anspruch 1 und 2, dadurch gekennzeichnet, daß das Molverhältnis der photochromen Verbindungen, definiert durch Formel (I), worin R₇ eine -NR₈R₉-Gruppe ist, zu den Verbindungen, ebenfalls definiert durch die Formel (I), worin R₇ Wasserstoff ist, durch eine Zahl innerhalb des Bereichs von 0,2 bis 1,5 umfaßt wird.

5. Verfahren nach Anspruch 1 oder 2 oder 3 oder 4, enthaltend 1,3,3-Trimethyl-6'-piperidino-spiro-[indolino-2,3'-(3H)-naphtho-(2,1-b)-(1,4)-oxazin].

6. Verfahren nach den Ansprüchen 1 bis 4, enthaltend 1,3,3-Trimethyl-6'-morpholino-spiro-[indolino-2,3'-(3H)-naphtho-(2,1-b)-(1,4)-oxazin].

7. Verfahren nach den Ansprüchen 1 bis 4, enthaltend 1,3,3,4,5-(oder 1,3,3,5,6-)Pentamethyl-6'-piperidino- spiro-[indolino-2,3'-(3H)-naphtho-(2,1-b)-(1,4)-oxazin].

8. Verfahren nach den Ansprüchen 1 bis 4, enthaltend 1,3,3-Trimethyl-6'-piperidino-9'-methoxy-spiro-[indolino-2,3'-(3H)-naphtho-(2,1-b)-(1,4)-oxazin].

9. Verfahren nach den Ansprüchen 1 bis 4, enthaltend 1,3,3,4,5-(oder 1,3,3,5,6-)Pentamethyl-spiro-[indolino-2,3'-(3H)-naphtho-(2,1-b)-(1,4)-oxazin].

10. Verfahren nach den Ansprüchen 1 bis 4, enthaltend 1,3,3-Trimethyl-spiro-[indolino-2,3'-(3H)-naphtho-(2,1-b)-(1,4)-oxazin].

11. Verfahren nach den Ansprüchen 1 bis 4, enthaltend 1,3,3-Trimethyl-9'-methoxy-spiro-[indolino-2,3'-(3H)-naphtho-(2,1-b)-(1,4)-oxazin].

12. Verfahren nach Anspruch 1, weiterhin umfassend einen UV-Stabilisator.

## Revendications (Revendications pour l'(les) Etat(s) contractant(s) suivant(s) : suivants : AT, BE, CH, DE, FR, GB, IT, LI, LU, NL, SE)

1. Composition photochrome comportant au moins deux composés photochromes, tous deux pouvant être représentés par la formule générale suivante (1) : dans laquelle
R₁ et R₂ représentent chacun, indépendamment, un atome d'hydrogène, un atome d'halogène choisi parmi F, CI et Br, ou un groupe choisi parmi les groupes alcoxy en C₁₋₅, nitro, cyano, et alkyle en C₁₋₅, linéaire ou ramifié, non substitué ou substitué par un atome d'halogène choisi parmi F, CI et Br,
ou par des groupes alcoxy en Ci -₅, alkylthio en Ci -₅, carboxyalkyle en Ci -₅ ou cyano ;
R₃ et R₄ représentent chacun, indépendamment, un groupe alkyle en C₁₋₅ linéaire ou ramifié, phényle
ou benzyle ; ou bien
R₃ et R₄, considérés conjointement avec l'atome de carbone auquel ils sont liés, forment un groupe cycloalkyle en C₅₋₈;
R₅ représente un groupe phényle, benzyle ou allyle, ou un groupe alkyle en C₁₋₅, linéaire ou ramifié, non substitué ou substitué par au moins un atome d'halogène choisi parmi F, CI et Br, ou par des groupes alcoxy en C₁₋₅ , alkylthio en C₁₋₅ , carboxylakyle en C₁₋₅ ou cyano ;
R₆ représente un atome d'hydrogène ou un atome d'halogène choisi parmi F, CI et Br, ou un groupe choisi parmi les groupes alcoxy en C₁₋₅, alkylthio en C₁₋₅, carboxyalkyle en C₁₋₅, cyano, et les groupes alkyle en C₁₋₅, linéaires ou ramifiés, non substitués ou substitués par au moins un atome d'halogène choisi parmi F, CI et Br, ou par des groupes alcoxy en C₁₋₅, alkylthio en C₁₋₅, carboxyalkyle en Ci -₅ ou cyano ; ou bien R₆ représente un noyau aromatique ou hétérocyclique condensé ;
R₆, quand il ne représente pas un atome d'hydrogène ou un noyau hétérocyclique ou aromatique condensé, peut être placé dans n'importe laquelle des positions 8', 9' et 10' du fragment naphtalénique
R₇ représente soit un atome d'hydrogène, soit un groupe -NR₈R₉ ; et
R₈ et Rg représentent chacun, indépendamment l'un de l'autre, un atome d'hydrogène ou un groupe alkyle en Ci -₅ linéaire ou ramifié, phényle ou benzyle, ou bien
R₈ et Rg, considérés conjointement avec l'atome d'azote auquel ils sont liés, forment une structure monocyclique ou polycyclique de 5 à 12 chaînons, comportant éventuellement un autre hétéroatome choisi parmi un atome d'oxygène et un atome d'azote ; et
X représente soit CH, soit N ;
composition dans laquelle, dans au moins l'un des composés photochromes définis par la formule (1), le substituant R₇ est constitué par un atome d'hydrogène, et dans au moins l'un des composés photochromes définis par la formule (1), le substituant R₇ est constitué par un groupe -NR₈R₉ dans lequel R₈ et R₉ sont définis comme indiqué plus haut.

2. Composition photochrome conforme à la revendication 1, caractérisée en ce que, dans au moins l'un des composés définis par la formule (1), en ce qui concerne les substituants :
R₁ et R₂ représentent chacun, indépendamment, un atome d'hydrogène ou un groupe méthyle ou méthoxy ;
R₃ et R₄ représentent chacun un groupe méthyle ou éthyle, ou bien, considérés conjointement, représentent le groupe cyclohexyle ;
R₅ représente un groupe alkyle en Ci -₅ ;
R₆ représente un atome d'hydrogène ou un groupe méthoxy ;
R₇ représente un groupe -NR₈R₉ dans lequel
R₈ et R₉ représentent, conjointement avec l'atome d'azote auquel ils sont liés, un groupe pipéridino, morpholino, pyrrolidinyle ou hexaméthylène-imino ; et
X représente soit -CH-, soit -N-.

3. Composition photochrome conforme aux revendications 1 et 2, caractérisée en ce que le rapport molaire des composés photochromes définis par la formule (I) et dans lesquels R₇ représente un groupe -NR₈R₉ aux composés définis eux aussi par la formule (I) et dans lesquels R₇ représente un atome d'hydrogène est un nombre situé dans l'intervalle allant de 0,1 à 9.

4. Composition photochrome conforme aux revendications 1 et 2, caractérisée en ce que le rapport molaire des composés photochromes définis par la formule (I) et dans lesquels R₇ représente un groupe -NR₈R₉ aux composés définis eux aussi par la formule (I) et dans lesquels R₇ représente un atome d'hydrogène est un nombre situé dans l'intervalle allant de 0,2 à 1,5.

5. Composition photochrome conforme à la revendication 1, 2, 3 ou 4, contenant de la 1,3,3-triméthyl-6'-pipéridino-spiro-[indolino-2,3'-(3H)-naphto-(2,1-b)-(1,4)-oxazine].

6. Composition photochrome conforme aux revendications 1 à 4, contenant de la 1,3,3-triméthyl-6'-morpholino-spiro-[indolino-2,3'-(3H)-naphto-(2,1-b)-(1,4)-oxazine].

7. Composition photochrome conforme aux revendications 1 à 4, contenant de la 1,3,3,4,5- ou 1,3,3,5,6-pentaméthyl-6'-pipéridino-spiro-[indolino-2,3'-(3H)-naphto-(2,1-b)-(1,4)-oxazine].

8. Composition photochrome conforme aux revendications 1 à 4, contenant de la 1,3,3-triméthyl-6'-pipéridino-9'-méthoxy-spiro-[indolino-2,3'-(3H)-naphto-(2,1-b)-(1,4)-oxazine].

9. Composition photochrome conforme aux revendications 1 à 4, contenant de la 1,3,3,4,5- ou 1,3,3,5,6-pentaméthyl-spiro-[indolino-2,3'-(3H)-naphto-(2,1-b)-(1,4)-oxazine].

10. Composition photochrome conforme aux revendications 1 à 4, contenant de la 1,3,3-triméthyl-spiro-[indolino-2,3'-(3H)-naphto-(2,1 -b)-(1,4)-oxazine].

11. Composition photochrome conforme aux revendications 1 à 4, contenant de la 1,3,3-triméthyl-9'-méthoxy-spiro-[indolino-2,3'-(3H)-naphto-(2,1-b)-(1,4)-oxazine].

12. Composition photochrome conforme aux revendications précédentes, contenant en outre un stabilisant UW.

13. Composition photochrome conforme à la revendication 12, caractérisée en ce que le stabilisant UV est une amine à encombrement stérique (HALS).

14. Article photochrome comprenant un polymère organique transparent et portant sur sa surface ou contenant dans sa masse une composition photochrome conforme aux revendications 1 à 10.

15. Article photochrome conforme à la revendication 14, dans lequel ledit polymère organique transparent est chosi parmi un poly(méthacrylate de méthyle), un poly(alcool vinylique), un poly(butyral de vinyle), une poly(vinyl-pirrolidone), un acétate-butyrate de cellulose, une résine époxy, une résine polysiloxane, une résine polyuréthane, un polycarbonate et un bis(allyl-carbonate) de poly-diéthylène-glycol.

## Revendications (Revendications pour l'(les) Etat(s) contractant(s) suivant(s) : suivant : ES)

1. Procédé de préparation d'une composition photochrome, caractérisé en ce qu'il comprend l'étape consistant à mélanger au moins deux composés photochromes, tous les deux pouvant être représentés par la formule générale suivante (1) : dans laquelle
R₁ et R₂ représentent chacun, indépendamment, un atome d'hydrogène, un atome d'halogène choisi parmi F, CI et Br, ou un groupe choisi parmi les groupes alcoxy en C₁₋₅, nitro, cyano, et alkyle en C₁₋₅, linéaire ou ramifié, non substitué ou substitué par un atome d'halogène choisi parmi F, CI et Br, ou par des groupes alcoxy en Ci -₅, alkylthio en Ci -₅, carboxyalkyle en Ci -₅ ou cyano ;
R₃ et R₄ représentent chacun, indépendamment, un groupe alkyle en C₁₋₅ linéaire ou ramifié, phényle ou benzyle ; ou bien
R₃ et R₄, considérés conjointement avec l'atome de carbone auquel ils sont liés, forment un groupe cycloalkyle en C₅₋₈ ;
R₅ représente un groupe phényle, benzyle ou allyle, ou un groupe alkyle en C₁₋₅ linéaire ou ramifié, non substitué ou substitué par au moins un atome d'halogène choisi parmi F, CI et Br, ou par des groupes alcoxy en C₁₋₅ , alkylthio en C₁₋₅ , carboxylakyle en C, -ₛ ou cyano ;
R₆ représente un atome d'hydrogène ou un atome d'halogène choisi parmi F, CI et Br, ou un groupe choisi parmi les groupes alcoxy en C₁₋₅, alkylthio en C₁₋₅, carboxyalkyle en C₁₋₅, cyano, et les groupes alkyle en C₁₋₅, linéaires ou ramifiés, non substitués ou substitués par au moins un atome d'halogène choisi parmi F, CI et Br, ou par des groupes alcoxy en C₁₋₅, alkylthio en C₁₋₅, carboxyalkyle en Ci -₅ ou cyano ; ou bien R₆ représente un noyau aromatique ou hétérocyclique condensé ;
R₆, quand il ne représente pas un atome d'hydrogène ou un noyau hétérocyclique ou aromatique condensé, peut être placé dans n'importe laquelle des positions 8', 9' et 10' du fragment naphtalénique
R₇ représente soit un atome d'hydrogène, soit un groupe -NR₈R₉ ; et
R₈ et R₉ représentent chacun, indépendamment l'un de l'autre, un atome d'hydrogène ou un groupe alkyle en Ci -₅ linéaire ou ramifié, phényle ou benzyle, ou bien
R₈ et Rg, considérés conjointement avec l'atome d'azote auquel ils sont liés, forment une structure monocyclique ou polycyclique de 5 à 12 chaînons, comportant éventuellement un autre hétéroatome choisi parmi un atome d'oxygène et un atome d'azote ; et
X représente soit CH, soit N ;
composition dans laquelle, dans au moins l'un des composés photochromes définis par la formule (1), le substituant R₇ est constitué par un atome d'hydrogène, et dans au moins l'un des composés photochromes définis par la formule (1), le substituant R₇ est constitué par un groupe -NR₈R₉ dans lequel R₈ et R₉ sont définis comme indiqué plus haut.

2. Procédé conforme à la revendication 1, caractérisé en ce que, dans au moins l'un des composés définis par la formule (1), en ce qui concerne les substituants :
R₁ et R₂ représentent chacun, indépendamment, un atome d'hydrogène ou un groupe méthyle ou méthoxy ;
R₃ et R₄ représentent chacun un groupe méthyle ou éthyle, ou bien, considérés conjointement, représentent le groupe cyclohexyle ;
R₅ représente un groupe alkyle en Ci -₅ ;
R₆ représente un atome d'hydrogène ou un groupe méthoxy ;
R₇ représente un groupe -NR₈R₉ dans lequel
R₈ et R₉ représentent, conjointement avec l'atome d'azote auquel ils sont liés, un groupe pipéridino, morpholino, pyrrolidinyle ou hexaméthylène-imino ; et
X représente soit -CH-, soit -N-.

3. Procédé conforme aux revendications 1 et 2, caractérisé en ce que le rapport molaire des composés photochromes définis par la formule (I) et dans lesquels R₇ représente un groupe -NR₈R₉ aux composés définis eux aussi par la formule (I) et dans lesquels R₇ représente un atome d'hydrogène est un nombre situé dans l'intervalle allant de 0,1 à 9.

4. Procédé conforme aux revendications 1 et 2, caractérisé en ce que le rapport molaire des composés photochromes définis par la formule (I) et dans lesquels R₇ représente un groupe -NR₈R₉ aux composés définis eux aussi par la formule (I) et dans lesquels R₇ représente un atome d'hydrogène est un nombre situé dans l'intervalle allant de 0,2 à 1,5.

5. Procédé conforme à la revendication 1, 2, 3 ou 4, caractérisé en ce que la composition contient de la 1,3,3-triméthyl-6'-pipéridino-spiro-[indolino-2,3'-(3H)-naphto-(2,1 -b)-(1,4)-oxazine].

6. Procédé conforme aux revendications 1 à 4, caractérisé en ce que la composition contient de la 1,3,3-triméthyl-6'-morpholino-spiro-[indolino-2,3'-(3H)-naphto-(2,1-b)-(1,4)-oxazine].

7. Procédé conforme aux revendications 1 à 4, caractérisé en ce que la composition contient de la 1,3,3,4,5- ou 1,3,3,5,6-pentaméthyl-6'-pipéridino-spiro-[indolino-2,3'-(3H)-naphto-(2,1-b)-(1,4)-oxazine].

8. Procédé conforme aux revendications 1 à 4, caractérisé en ce que la composition contient de la 1,3,3-triméthyl-6'-pipéridino-9'-méthoxy-spiro-[indolino-2,3'-(3H)-naphto-(2,1-b)-(1,4)-oxazine].

9. Procédé conforme aux revendications 1 à 4, caractérisé en ce que la composition contient de la 1,3,3,4,5- ou 1,3,3,5,6-pentaméthyl-spiro-[indolino-2,3'-(3H)-naphto-(2,1-b)-(1,4)-oxazine].

10. Procédé conforme aux revendications 1 à 4, caractérisé en ce que la composition contient de la 1,3,3-triméthyl-spiro-[indolino-2,3'-(3H)-naphto-(2,1-b)-(1,4)-oxazine].

11. Procédé conforme aux revendications 1 à 4, caractérisé en ce que la composition contient de la 1,3,3-triméthyl-9'-méthoxy-spiro-[indolino-2,3'-(3H)-naphto-(2,1-b)-(1,4)-oxazine].

12. Procédé conforme à la revendication 1, caractérisé en ce qu'il comporte en outre l'addition d'un stabilisant UV.
